



US005897426A

# United States Patent [19]

Somekh

[11] Patent Number: 5,897,426

[45] Date of Patent: Apr. 27, 1999

[54] **CHEMICAL MECHANICAL POLISHING WITH MULTIPLE POLISHING PADS**[75] Inventor: **Sasson Somekh**, Los Altos Hills, Calif.[73] Assignee: **Applied Materials, Inc.**, Santa Clara, Calif.[21] Appl. No.: **09/066,271**[22] Filed: **Apr. 24, 1998**[51] Int. Cl.<sup>6</sup> ..... **B24B 7/22**[52] U.S. Cl. ..... **451/41; 451/57**[58] Field of Search ..... **451/41, 36, 37, 451/57, 288, 287; 438/692, 693**[56] **References Cited**

## U.S. PATENT DOCUMENTS

|           |         |                     |         |
|-----------|---------|---------------------|---------|
| 5,244,534 | 9/1993  | Yu et al. ....      | 156/636 |
| 5,395,801 | 3/1995  | Doan et al. ....    | 437/225 |
| 5,676,857 | 10/1997 | Landers et al. .... | 451/57  |
| 5,718,618 | 2/1998  | Guckel et al. ....  | 451/41  |
| 5,823,855 | 10/1998 | Robinson ....       | 451/41  |

Primary Examiner—Robert A. Rose

Attorney, Agent, or Firm—Fish &amp; Richardson

[57] **ABSTRACT**

In chemical mechanical polishing, a substrate is planarized with one or more fixed-abrasive polishing pads. Then the substrate is polished with a standard polishing pad to remove scratch defects created by the fixed-abrasive polishing pads.

**18 Claims, 4 Drawing Sheets**

**FIG.\_1**

**FIG.\_2A****FIG.\_2B**

**FIG. 3A****FIG. 3B****FIG. 3C**



***FIG.\_3D***



***FIG.\_3E***

## CHEMICAL MECHANICAL POLISHING WITH MULTIPLE POLISHING PADS

### BACKGROUND

The present invention relates generally to chemical mechanical polishing of substrates, and more particularly to polishing with fixed-abrasive polishing pads.

Integrated circuits are typically formed on substrates, particularly silicon wafers, by the sequential deposition of conductive, semiconductive or insulative layers. After each layer is deposited, the layer is etched to create circuitry features. As a series of layers are sequentially deposited and etched, the outer or uppermost surface of the substrate, i.e., the exposed surface of the substrate, becomes increasingly non-planar. This non-planar outer surface presents a problem for the integrated circuit manufacturer. Therefore, there is a need to periodically planarize the substrate surface to provide a relatively flat surface. However, in some fabrication processes, planarization of the outer layer should not expose underlying layers.

Chemical mechanical polishing (CMP) is one accepted method of planarization. This planarization method typically requires that the substrate be mounted on a carrier or polishing head. The exposed surface of the substrate is placed against a rotating polishing pad. The polishing pad may be either a "standard" pad or a fixed-abrasive pad. A fixed-abrasive pad has abrasive particles held in a containment media, whereas a standard pad has a durable surface, without embedded abrasive particles. The carrier head provides a controllable load, i.e., pressure, on the substrate to push it against the polishing pad. A polishing slurry, including at least one chemically-reactive agent, and abrasive particles if a standard pad is used, is supplied to the surface of the polishing pad.

An effective CMP process not only provides a high polishing rate, but also provides a substrate surface which is finished (lacks small-scale roughness) and flat (lacks large-scale topography). The polishing rate, finish and flatness are determined by the pad and slurry combination, the relative speed between the substrate and pad, and the force pressing the substrate against the pad.

A reoccurring problem with fixed-abrasive pads is scratching of the substrate surface. Specifically, some CMP processes that use fixed-abrasive pads create shallow grooves, e.g., on the order of 500 angstroms deep, in the substrate surface. These grooves render the substrate finish unsuitable for integrated circuit fabrication, lowering the process yield.

### SUMMARY

In one aspect, the invention is directed to a method of polishing a substrate. The process includes chemical mechanical polishing the substrate with a fixed-abrasive polishing pad until it is substantially planarized, and chemical mechanical polishing the substrate with a non-fixed-abrasive polishing pad to remove any scratches.

Implementations of the invention may include the following. The fixed-abrasive polishing pad may be located at a first polishing station of a polishing apparatus, and the non-fixed-abrasive polishing pad may be located at a second polishing station of the polishing apparatus. The substrate may be chemical mechanical polished with a second fixed-abrasive polishing pad or a second non-fixed-abrasive polishing pad at a third polishing station, e.g., before polishing the substrate at the second polishing station. A first polishing

liquid may be supplied to the first polishing station, a second polishing liquid may be supplied to the second polishing station, and a third polishing liquid may be supplied to the third polishing station. The first polishing liquid may have a different pH than the second polishing liquid. The second polishing liquid may contain abrasive particles. The fixed-abrasive polishing pad may include an upper layer that includes abrasive grains held in a binder material, and a lower layer selected from the group consisting of polymeric film, paper, cloth, and metallic film. The non-fixed-abrasive polishing pad may include a first layer including polyurethane and a second layer including compressed felt fibers, or a layer composed of a poromeric material.

In another aspect, the invention is directed to a method of forming a planarized layer on a substrate. A layer is formed on a non-planar surface of the substrate. The layer is chemical mechanical polished with a fixed-abrasive polishing pad until a residual layer remains over the surface, and the residual layer is chemical mechanical polished with a non-fixed-abrasive polishing pad to remove any scratches. The residual layer has a thickness equal to or greater than the depth of any scratches therein.

Implementations of the invention may include the following. The residual layer may have a thickness approximately equal to the depth of any scratches, e.g., about 100 to 1000 angstroms. Polishing with the non-fixed-abrasive polishing pad may cease when a layer having a target thickness, e.g., 300 to 1000 angstroms, remains over the non-planar surface.

Advantages of the invention may include the following. Scratching of the substrate is reduced or eliminated, thereby increasing process yield.

Other features and advantages will be apparent from the following description, including the drawings and claims.

### BRIEF DESCRIPTION OF THE DRAWINGS

FIG. 1 is a schematic exploded perspective view of a chemical mechanical polishing apparatus.

FIG. 2A is a schematic cross-sectional view of the first polishing station of the CMP apparatus of FIG. 1.

FIG. 2B is a schematic cross-sectional view of the final polishing station of the CMP apparatus of FIG. 1.

FIGS. 3A-3E are schematic cross sectional views of a substrate illustrating the method of the present invention.

### DETAILED DESCRIPTION

Referring to FIG. 1, one or more substrates **10** will be polished by a chemical mechanical polishing apparatus **20**. A description of polishing apparatus **20** may be found in U.S. Pat. No. 5,738,574, the entire disclosure of which is incorporated herein by reference. Polishing apparatus **20** includes a lower machine base **22** with a table top **23** mounted thereon and a removable outer cover (not shown). Table top **23** supports a series of polishing stations, including a first polishing station **25a**, a second polishing station **25b**, and a final polishing station **25c**, and a transfer station **27**. Transfer station **27** forms a generally square arrangement with the three polishing stations **25a**, **25b** and **25c**. Transfer station **27** serves multiple functions, including receiving individual substrates **10** from a loading apparatus (not shown), washing the substrates, loading the substrates into carrier heads, receiving the substrates from the carrier heads, washing the substrates again, and finally, transferring the substrates back to the loading apparatus.

Each polishing station includes a rotatable platen **30** on which is placed a polishing pad. The first and second stations

**25a** and **25b** may include a fixed-abrasive pad **100**, whereas the final polishing station may include a standard pad **110**. If substrate **10** is an "eight-inch" (200 millimeter) or "twelve-inch" (300 millimeter) diameter disk, then the platens and polishing pads will be about twenty inches or thirty inches in diameter, respectively. Each platen **30** may be a rotatable aluminum or stainless steel plate connected to a platen drive motor (not shown). For most polishing processes, the platen drive motor rotates platen **30** at thirty to two hundred revolutions per minute, although lower or higher rotational speeds may be used.

Polishing station **25c** may include a pad conditioner apparatus **40**. Pad conditioner apparatus **40** has a rotatable arm **42** holding an independently-rotating conditioner head **44** and an associated washing basin **46**. The pad conditioner apparatus **40** maintains the condition of the polishing pad so that it will effectively polish substrates. Polishing stations **25a** and **25b** do not require a pad conditioner apparatus because fixed-abrasive pads generally do not require conditioning. However, as illustrated, each polishing station may include a conditioning station in the event that the CMP apparatus is used with other pad configurations. (e.g., silica particles for oxide polishing) and a chemically-reactive agent (e.g., potassium hydroxide for oxide polishing). The concentration of agents in the polishing liquids may be different. Specifically, the pH of polishing liquid **50a** may differ from the pH of polishing liquid **50b**.

Each slurry/rinse arm may include two or more slurry supply tubes to provide slurry to the surface of the polishing pad. Sufficient slurry may be provided to cover and wet the entire polishing pad. Each slurry/rinse arm **52** also includes several spray nozzles (not shown) which provide a high-pressure rinse of the polishing pad at the end of each polishing and conditioning cycle.

Two or more intermediate washing stations **55a** and **55b** may be positioned between neighboring polishing stations **25a**, **25b** and **25c**. The washing stations rinse the substrates after they leave the polishing stations.

A rotatable multi-head carousel **60** is positioned above lower machine base **22**. Carousel **60** is supported by a center post **62** and is rotated thereon about a carousel axis **64** by a carousel motor assembly located within machine base **22**. Center post **62** supports a carousel support plate **66** and a cover **68**. Carousel **60** includes four carrier head systems **70a**, **70b**, **70c**, and **70d**. Three of the carrier head systems receive and hold substrates, and polish them by pressing them against the polishing pads on the platens of polishing stations **25a**–**25c**. One of the carrier head systems receives a substrate from and delivers a substrate to transfer station **27**.

The four carrier head systems **70a**–**70d** are mounted on carousel support plate **66** at equal angular intervals about carousel axis **64**. Center post **62** allows the carousel motor to rotate carousel support plate **66** and to orbit carrier head systems **70a**–**70d** and the substrates attached thereto about carousel axis **64**.

Each carrier head system **70a**–**70d** includes a carrier or carrier head **80**. A carrier drive shaft **74** connects a carrier head rotation motor **76** (shown by the removal of one quarter of cover **68**) to carrier head **80** so that each carrier head **80** can independently rotate about its own axis. There is one carrier drive shaft and motor for each head. In addition, each carrier head **80** independently laterally oscillates in a radial slot **72** formed in carousel support plate **66**. A slider (not shown) supports each drive shaft in its associated radial slot. A radial drive motor (not shown) may move the slider to laterally oscillate the carrier head.

The carrier head **80** performs several mechanical functions. Generally, the carrier head holds the substrate against the polishing pad, evenly distributes a downward pressure across the back surface of the substrate, transfers torque from the drive shaft to the substrate, and ensures that the substrate does not slip out from beneath the carrier head during polishing operations.

The carrier head **80** may include a flexible membrane (not shown) which provides a substrate receiving surface. A description of a suitable carrier head **80** may be found in U.S. patent application Ser. No. 08/745,679, entitled a CARRIER HEAD WITH a FLEXIBLE MEMBRANE FOR a CHEMICAL MECHANICAL POLISHING SYSTEM, filed Nov. 8, 1996, by Steven M. Zuniga et al., assigned to the assignee of the present invention, the entire disclosure of which is incorporated herein by reference.

Referring to FIG. 2A, an aperture or hole **34** is formed in each platen **30** and a transparent window **36** is formed in a portion of the polishing pad overlying the hole. The transparent window **36** may be constructed as described in U.S. patent application Ser. No. 08/689,930, entitled METHOD OF FORMING A TRANSPARENT WINDOW IN A POLISHING PAD FOR A CHEMICAL MECHANICAL POLISHING APPARATUS by Manoocher Birang, et al., filed Aug. 26, 1996, and assigned to the assignee of the present invention, the entire disclosure of which is incorporated herein by reference. The hole **34** and transparent window **36** are positioned such that they have a "view" of substrate **10** during a portion of the platen's rotation, regardless of the translational position of the polishing head. A laser interferometer **90** is located below platen **30**. The laser interferometer includes a laser **94** and a detector **96**. The laser generates a collimated laser beam **92** which propagates through transparent window **36** to impinge upon the exposed surface of substrate **10**.

Laser **94** is activated to generate laser beam **92** during a time when hole **34** is adjacent substrate **10**. In operation, CMP apparatus **20** uses laser interferometer **90** to determine the amount of material removed from the surface of the substrate, or to determine when the surface has become planarized. A general purpose programmable digital computer **98** may be connected to laser **94** and detector **96**. Computer **98** may be programmed to activate the laser when the substrate overlies the window, to store measurements from the detector, to display the measurements on an output device **93**, and to detect the polishing endpoint, as described in aforementioned U.S. patent application Ser. No. 08/689,930.

Still referring to FIG. 2A, at first and second polishing stations **25a** and **25b**, the platen supports a fixed-abrasive polishing pad **100** having a polishing surface **102**. The fixed-abrasive polishing pad **100** includes an upper layer **104** and a lower layer **106**. Lower layer **106** may be attached to platen **30** by a pressure-sensitive adhesive layer **108**. Upper layer **104** typically will be a 5–200 mil thick abrasive composite layer, composed of abrasive grains held or embedded in a binder material. The abrasive grains may have a particle size between about 0.1 and 1500 microns, and have a Mohs' hardness of at least 8. Examples of such grains include fused aluminum oxide, ceramic aluminum oxide, green silicon carbide, silicon carbide, chromia, alumina zirconia, diamond, iron oxide, ceria, cubic boron nitride, garnet and combinations thereof. The binder material may be derived from a precursor which includes an organic polymerizable resin which is cured from the binder material. Examples of such resins include phenolic resins, urea-formaldehyde resins, melamine formaldehyde resins,

acrylated urethanes, acrylated epoxies, ethylenically unsaturated compounds, aminoplast derivatives having at least one pendant acrylate group, isocyanurate derivatives having at least one pendant acrylate group, vinyl ethers, epoxy resins, and combinations thereof. Lower layer **106** typically will be a 25–200 mil thick backing layer, composed of a material such as a polymeric film, paper, cloth, a metallic film or the like.

Fixed-abrasive polishing pads are described in detail in the following U.S. patents, all of which are incorporated by reference: U.S. Pat. No. 5,152,917, issued on Oct. 6, 1992, and entitled STRUCTURED ABRASIVE ARTICLE; U.S. Pat. No. 5,342,419, issued on Aug. 30, 1994, and entitled ABRASIVE COMPOSITES HAVING A CONTROLLED RATE OF EROSION, ARTICLES INCORPORATING SAME, AND METHODS OF MAKING AND USING SAME; U.S. Pat. No. 5,368,619, issued on Nov. 29, 1994, and entitled REDUCED VISCOSITY SLURRIES, ABRASIVE ARTICLES MADE THEREFROM AND METHODS OF MAKING SAID ARTICLES; and U.S. Pat. No. 5,378,251, issued on Jan. 3, 1995, and entitled ABRASIVE ARTICLES AND METHOD OF MAKING AND USING SAME. Fixed-abrasive pads are available from 3M Corporation of Minneapolis, Minn.

Referring to FIG. 2B, at final polishing station **25c**, the platen may support a standard polishing or “non-fixed-abrasive” pad **110**, i.e., a polishing pad that does not have embedded abrasive particles, having a generally smooth polishing surface **112** and including a single soft layer **114**. Layer **114** may be attached to platen **30** by a pressure-sensitive adhesive layer **118**. Layer **114** may be composed of a napped poromeric synthetic material. A suitable soft polishing pad is available from Rodel, Inc., of Newark, Del., under the trade name Politex. Polishing pad **110** may be embossed or stamped with a pattern to improve distribution of slurry across the face of the substrate. Alternatively, polishing pad **110** may be a standard two-layer pad in which the upper layer has a durable roughened surface and is harder than the lower layer. For example, the upper layer of the two-layer pad may be composed of microporous polyurethane or polyurethane mixed with a filler, whereas the lower layer may be composed of compressed felt fibers leached with urethane. Both the upper and lower layers may be approximately fifty mils thick. A two-layer standard pad, with the upper layer composed of IC-1000 and the lower layer composed of SUBA-4, is available from Rodel (IC-1000 and SUBA-4 are product names of Rodel, Inc.). Polishing station **25c** may otherwise be identical to polishing stations **25a** and **25b**.

FIGS. 3A–3E illustrate the process of chemical-mechanically polishing a layer, such as an insulative layer. Although an insulative layer is shown and discussed, the invention may also be applicable to polishing of metallic and semiconductive layers. As shown in FIG. 3A, substrate **10** includes a metal layer **14**, such as copper or tungsten, disposed on a silicon wafer **12**. The metal layer **14** is either patterned or disposed on a patterned underlying layer so that it has a non-planar outer surface. An insulative layer **16**, such as silicon dioxide, is disposed over metal layer **14**. The outer surface of insulative layer **16** almost exactly replicates the underlying structures of metal layer **14**, creating a series of peaks and valleys so that the exposed surface of the substrate is non-planar.

As discussed above, one purpose of planarization is to polish insulative layer **16** until its surface is flat and finished. Unfortunately, one problem with polishing with fixed-abrasive pads is the creation of scratches in the outer surface

of the resulting substrate. Furthermore, as discussed above, the underlying metal layer should not be exposed. Thus, polishing should cease when an insulative layer having a target thickness **T** remains over the metal layer. The target thickness **T** may be about 300 to 1000 angstroms.

Referring to FIG. 3B, substrate **10** is initially polished at polishing stations **25a** and **25b** with polishing liquid **50a** and one or more fixed-abrasive polishing pads **100**. As shown in FIG. 3C, the substrate is polished until insulative layer **16** is substantially planarized, i.e., the large-scale topography such as the peaks and valleys have been substantially removed, and a residual film **18** having a thickness **D** remains over the target thickness. The thickness of the residual film is equal to or greater than the depth of the scratches **120**. Specifically, the thickness **D** may be about 100 to 1000 angstroms, e.g., up to about 500 angstroms. The laser interferometer **90** (see FIG. 2A) may be used to determine when the substrate has been polished until a residual layer with the desired thickness remains.

Then, referring to FIG. 3D, the substrate is polished at final polishing station **25c** using polishing liquid **50b** and standard polishing pad **110**. The substrate is polished using the soft polishing pad until residual film **18** is removed and an insulative layer of the target thickness **T** remains over the metal layer, as shown in FIG. 3E. The scratches caused by polishing with the fixed-abrasive pads at polishing stations **25a** and **25b** are removed by polishing away the residual film with standard polishing pad **110**. Thus, scratch defects are reduced and process yields increased. The majority of the insulative layer is planarized by use of the fixed-abrasive polishing pads, which do not require a slurry that contains abrasive particles or conditioning. Furthermore, in contrast to polishing methods in which only buffing is performed at the final station and the final station lies idle while polishing is performed at the first and second stations, the polishing liquid **50b** may contain abrasive particles and a part of the insulative layer may be removed at the final polishing station, thus decreasing the polishing time at the first and second polishing stations and further increasing throughput. In addition, polishing with the soft pad helps remove polishing debris from the substrate surface.

Alternately, the substrate may be initially polished at polishing station **25a** with polishing liquid **50a** and a fixed-abrasive polishing pad **100**, and then polished at polishing stations **25b** and **25c** with standard polishing pads **110**. For example, particularly in metal polishing, copper layer may be polished with the fixed-abrasive pad at the first polishing station, the barrier layer may be polished with a standard polishing pad (e.g., a two-layer pad) at the second polishing station, and the scratches may be removed with another standard polishing pad (e.g., a soft pad) at the third polishing station. Different polishing liquids may be supplied to the three polishing stations.

The invention is not limited to the embodiment depicted and described. Rather, the scope of the invention is defined by the appended claims.

What is claimed is:

1. A method of polishing a substrate, comprising: chemical mechanical polishing the substrate with a fixed-abrasive polishing pad until it is substantially planarized; and chemical mechanical polishing the substrate with a non-fixed-abrasive polishing pad to remove any scratches.
2. The method of claim 1, wherein the fixed-abrasive polishing pad is located at a first polishing station of a polishing apparatus and the non-fixed-abrasive polishing pad is located at a second polishing station of the polishing apparatus.

3. The method of claim 2, further comprising chemical mechanical polishing the substrate with a second fixed-abrasive polishing pad at a third polishing station before polishing the substrate at the second polishing station.

4. The method of claim 2, further comprising chemical mechanical polishing the substrate with a second non-fixed-abrasive polishing pad at a third polishing station.

5. The method of claim 4, further comprising supplying a first polishing liquid to the first polishing station, supplying a second polishing liquid to the second polishing station, and supplying a third polishing liquid to the third polishing station.

6. The method of claim 1, further comprising supplying a first polishing liquid to the fixed-abrasive polishing pad and supplying a second polishing liquid to the non-fixed-abrasive polishing pad.

7. The method of claim 6, wherein the first polishing liquid has a different pH than the second polishing liquid.

8. The method of claim 6, wherein the second polishing liquid contains abrasive particles.

9. The method of claim 1, wherein the fixed-abrasive polishing pad includes an upper layer and a lower layer.

10. The method of claim 9, wherein the upper layer of the fixed-abrasive polishing pad includes abrasive grains held in a binder material.

11. The method of claim 9, wherein the lower layer of the fixed-abrasive polishing pad is selected from the group consisting of polymeric film, paper, cloth, and metallic film.

12. The method of claim 1, wherein the non-fixed-abrasive polishing pad includes a first layer including polyurethane and a second layer including compressed felt fibers.

13. The method of claim 1, wherein the non-fixed-abrasive polishing pad includes a layer composed of a poromeric material.

14. A method of forming a planarized layer on a substrate, comprising:

forming a layer on a non-planar surface of the substrate; chemical mechanical polishing the layer with a fixed-abrasive polishing pad until a residual layer remains over the surface, the residual layer having a thickness equal to or greater than the depth of any scratches therein; and

chemical mechanical polishing the residual layer with a non-fixed-abrasive polishing pad to remove any scratches.

15. The method of claim 14, wherein the residual layer has a thickness approximately equal to the depth of any scratches.

16. The method of claim 14, wherein the residual layer has a thickness of about 100 to 1000 angstroms.

17. The method of claim 14, wherein chemical mechanical polishing with the non-fixed-abrasive polishing pad ceases when a layer having a target thickness remains over the non-planar surface.

18. The method of claim 17, wherein the target thickness is about 300 to 1000 angstroms.

\* \* \* \* \*